

# UNITED STATES PATENT OFFICE.

ARCHIBALD O. MASON, OF CHICAGO, ILLINOIS.

## ALUMINUM ALLOY.

1,305,300.

Specification of Letters Patent. Patented June 3, 1919.

No Drawing.

Application filed July 1, 1918. Serial No. 242,838.

To all whom it may concern:

Be it known that I, ARCHIBALD O. MASON, a citizen of the United States of America, and a resident of Chicago, county of Cook, 5 and State of Illinois, have invented certain new and useful Improvements in Aluminum Alloys, of which the following is a specification.

The main objects of this invention are to 10 provide an improved aluminum alloy obtained by the addition of a comparatively small quantity of other metals which, without impairing the strength and lightness of the product, impart to it other qualities 15 which make it superior to other aluminum alloys for general use in the formation of castings; and to provide an improved compound of aluminum, copper, and zinc which is peculiarly suitable for making castings 20 and at the same time more ductile and more easily machined than the aluminum alloys which have been heretofore commonly used.

Aluminum has recently come into great demand for castings where strength combined with low weight is desired. The most extensive use of aluminum at the present time is for the castings for automobile and aeroplane motors, where great strength is required, but where lightness and compactness 30 are also very essential.

Heretofore there has been and still is being marketed an aluminum alloy for this purpose which has come to be known in the trade as "standard." This alloy generally 35 comprises 92 per cent. aluminum and 8 per cent. copper. Notwithstanding the rather extensive use of this "standard" alloy, it has certain objections as to its lack of ductility and its poor machining qualities.

It is the purpose of the present invention 40 to provide an aluminum alloy which possesses substantially all of the valuable characteristics of the "standard" aluminum with regard to strength and lightness, but which overcomes the aforesaid objectionable characteristics. To that end, the present alloy involves reducing the amount of copper as 45 compared with the "standard" alloy and adding a small quantity of zinc. The proportions which have been found to produce 50 the most satisfactory results are substantially 91½ per cent. aluminum, 6½ per cent. copper, and 2 per cent. zinc.

The reduction in the amount of copper tends to increase the ductility of the alloy, 55 and the addition of the zinc tends to make the machining thereof much easier, and the result of said machining is a much smoother and more finished surface than is the case with the "standard" alloy. The product is 60 capable of use for castings to the same extent that said "standard" alloy has been found practical, and because of these additional advantages, is much more suitable for many 65 purposes.

I claim:

1. An alloy of aluminum, copper, and zinc, substantially in the proportions of 91½ per cent. aluminum, 6½ per cent copper, and 2 per cent. zinc.
2. An alloy of about 91½ per cent. of aluminum, about 6½ per cent. of copper, and a small part of zinc sufficient to adapt it for good machining, the zinc content ranging from 1 to 2 per cent.

Signed at Chicago this 26th day of June, 1918.

ARCHIBALD O. MASON.